

1

2,817,586

## RESISTOR ALLOY

John Harry Jackson, Columbus, Ohio, and James F. Kavanaugh, Westport, Conn., assignors, by mesne assignments, to The C. O. Jelliff Manufacturing Corporation, Southport, Conn., a corporation of Connecticut

No Drawing. Application October 31, 1956,  
Serial No. 619,401

5 Claims. (Cl. 75—171)

This invention relates to resistor alloys and is particularly directed to the provision of an improved alloy for fabrication into wires for wire-wound electrical resistance elements. The invention provides an improved alloy amenable to production and fabrication on a commercial scale and by commercially practical procedures, which can consistently be formed into wires and other articles having a high electrical resistivity and a very low (and generally positive) temperature coefficient of resistivity.

The alloy of this invention consists essentially of 8% to 28% chromium (all percentage composition figures herein are by weight), 15% to 36% manganese, 0.1% to 4% molybdenum, 0.1% to 3% aluminum, 1/2% to 5% cobalt, and the balance nickel. Such an alloy, in the annealed condition, possesses an electrical resistivity of approximately 800 ohms per circular mil foot and has a temperature coefficient of resistivity within the range +0.00001 to -0.00001 ohm per ohm per °C.

Preferably, electrical resistance alloys according to the invention fall within the somewhat narrower composition range of 15% to 25% chromium, 15% to 25% manganese, 1% to 3% molybdenum, 0.1% to 1.0% aluminum, 1/2% to 5% cobalt, and the balance nickel, the nickel preferably constituting from 50% to 70% of the alloy. The resistivity of these alloys is generally near or above 800 ohms per circular mil foot, while the temperature coefficient of resistivity is at a value between +0.00001 and -0.00001. A particularly advantageous alloy according to the invention is one consisting essentially of about 20% chromium, about 18% manganese, about 1.5% molybdenum, about 0.25% aluminum, about 1.5% cobalt, and the balance nickel.

Alloys composed essentially of chromium, manganese and molybdenum within the ranges stated above, and the balance nickel, have been produced and used heretofore as electrical resistance alloys. Indeed, such alloys can be heat treated (solution annealed and then aged) to develop very high electrical resistivity, in the neighborhood of 1000 ohms per circular mil foot. However, it is very difficult under commercial manufacturing conditions to produce wires of such alloys which consistently possess electrical resistivities above about 750 ohms per circular mil foot. Moreover, it is difficult to avoid embrittlement of wires of such alloys in their manufacture when they are heat treated (solution annealed and then aged) to possess high electrical resistivity (i. e. above about 750 ohms per circular mil foot). In addition, wires fabricated commercially of such alloys generally possess a temperature coefficient of resistivity substantially exceeding 10 parts per million.

The present invention is based on the discovery that by adding aluminum and cobalt in the ranges stated above to the base alloy of chromium, manganese, nickel and molybdenum in the amounts stated above, a notable improvement in the electrical resistivity and a notable narrowing of the range of the temperature coefficient of resistivity of the alloy is secured. The aluminum addition favorably influences the resistivity, while additions of co-

2

balt have been found to constitute an effective means of controlling the temperature coefficient of resistivity of the alloy. Such alloys, containing aluminum and cobalt, can be readily and consistently produced and fabricated into wires by conventional commercial techniques, which wires consistently possess, as annealed, electrical resistivities of about 800 ohms per circular mil foot. Furthermore, the aluminum- and cobalt-bearing alloys of this invention have a very small temperature coefficient of resistivity, less than 10 parts per million, and generally of positive sign (i. e., resistivity increases slightly with increase in temperature).

Optimum properties are developed in alloys of this invention by annealing the metal at a temperature in the range from 1500° F. to 2100° F., and preferably in the upper portion of this range, that is, from 1700° F. to 2100° F. The time required for the annealing treatment depends on the annealing temperature, ranging from as much as 100 hours at a temperature of 1500° F. to as little as two seconds (in the case of fine wires) at a temperature of 2100° F. The time required for annealing is of course also dependent on the physical size of the article being treated, being much less for small diameter wires than for large diameter bars or rods. It is also to some extent dependent on the prior history of the alloy. For example, if the alloy is in the as-cast condition, the annealing time must be longer than if the alloy has undergone some measure of mechanical working. In the annealed condition, the metal is readily worked by conventional cold rolling and cold drawing operations to produce strips and wires that are subsequently to be fabricated into electrical resistance devices.

Following is an example of this invention: An alloy composed essentially of 19.5% chromium, 18.5% manganese, 1.5% molybdenum, 1.0% aluminum, 3.0% cobalt, and the balance nickel was melted and cast, forged into small bars about 1/2 inch square in cross section, swaged to 1/4-inch diameter rod, and then cold drawn into the form of round wire about 0.01 inch in diameter. The wire was annealed by heating it at 1800° F. for approximately 1/2 hour, and then was air cooled to room temperature. The resulting wire had an electrical resistivity of 789 ohms per circular mil foot, and a temperature coefficient of resistivity of +0.000004. This wire was readily formed into resistor coils and other shapes.

In preparing the alloys of this invention, it is the usual practice to add silicon in amounts of about 0.2% as a deoxidizer. This addition, together with silicon from the original charge, often results in a residual silicon content of from 0.35% to 0.4%, without affecting the properties of the alloy. In a similar way, titanium in amounts up to about 0.2% is often added to effect grain refinement. The presence or absence of such elements is immaterial to the alloys of this invention.

Other examples of alloys according to this invention are set forth in the following table:

|    | Composition <sup>1</sup> |      |      |      |     | Resistivity <sup>2</sup><br>in ohms per circular mil foot | T. C.,<br>p. p. m. |
|----|--------------------------|------|------|------|-----|-----------------------------------------------------------|--------------------|
|    | Cr                       | Mn   | Co   | Mo   | Al  |                                                           |                    |
| 60 | 19.8                     | 18.0 | 1.31 | 1.28 | .20 | 800                                                       | +2                 |
|    | 19.81                    | 19.0 | 1.58 | 1.57 | .20 | 802                                                       | -3                 |
|    | 19.5                     | 19.2 | 1.48 | 1.75 | .21 | 812                                                       | -3                 |
|    | 19.6                     | 17.6 | 1.26 | 1.46 | .12 | 800                                                       | +9                 |

<sup>1</sup> Composition—balance nickel plus impurities, deoxidizer, and grain refiner.

<sup>2</sup> Resistivity—in ohms per circular mil foot.

<sup>3</sup> Temperature coefficient of resistivity—in parts per million.

We claim:

70 1. An electrical resistance alloy consisting essentially of 8% to 28% chromium, 15% to 36% manganese, 0.1%

to 4% molybdenum, 0.1% to 3% aluminum, 1/2% to 5% cobalt, and the balance nickel.

2. An electrical resistance alloy consisting essentially of 15% to 25% chromium, 15% to 25% manganese, 1% to 3% molybdenum, 0.1% to 1.0% aluminum, 1/2% to 5% cobalt, and the balance nickel, said nickel constituting 50% to 70% of the alloy.

3. An electrical resistance alloy consisting essentially of about 20% chromium, about 18% manganese, about 1.5% molybdenum, about 0.25% aluminum, about 1.5% cobalt, and the balance nickel.

4. An electrical resistance alloy consisting essentially of 8% to 28% chromium, 15% to 36% manganese, 0.1% to 4% molybdenum, 0.1% to 3% aluminum, 1/2% to 5% cobalt, and the balance nickel, said alloy being in the 15

annealed condition and having an electrical resistivity of approximately 800 ohms per circular mil foot and having a temperature coefficient of resistivity within the range from +0.00001 to -0.00001.

5. An electrical resistance alloy consisting essentially of 15% to 25% chromium, 15% to 25% manganese, 1% to 3% molybdenum, 0.1% to 1% aluminum, 1/2% to 5% cobalt, and the balance nickel, said nickel constituting 50% to 70% of the alloy, and said alloy being in the annealed condition and having an electrical resistivity of approximately 800 ohms per circular mil foot and having a temperature coefficient of resistivity from +0.00001 to -0.00001.

No references cited.